

A. E. SCHUTTE.  
STREET PAVEMENT OR ROADWAY.  
APPLICATION FILED MAY 3, 1905.

912,898.

Patented Feb. 16, 1909.



Fig. 1.



Fig. 2.



Fig. 3.

WITNESSES:

Robert E. Brewer

Martin V. Foley

INVENTOR:

August E. Schutte

by his attorney  
Clarke, Raymond & Cook.

# UNITED STATES PATENT OFFICE.

AUGUST E. SCHUTTE, OF BOSTON, MASSACHUSETTS.

## STREET PAVEMENT OR ROADWAY.

No. 912,898

Specification of Letters Patent.

Patented Feb. 16, 1902.

Application filed May 3, 1905. Serial No. 253,697.

To all whom it may concern:

Be it known that I, AUGUST E. SCHUTTE, a subject of William, Emperor of Germany, having taken out my first naturalization 5 papers as citizen of the United States, and now residing in Boston, county of Suffolk, and State of Massachusetts, have invented a new and useful Improvement in Street Pavements or Roadways, of which the following is a full, clear, and exact description, reference being had to the accompanying drawings, forming a part of this specification, in explaining its nature.

The invention relates to the construction 15 of a wearing surface of a sheet pavement upon a suitable foundation—concrete, or of any other kind. This wearing surface is made of a mixture of stones, sand and bitumen.

20 It has been the special object of my invention to devise a means whereby a stable wearing surface for a pavement of bituminous concrete may be constructed of as few grades of crushed stone as possible, thus 25 eliminating much of the labor and expense of screening the stone and much of the necessity of measuring by weight or bulk various grades of mineral components hitherto used in various proportions in the 30 construction of this class of pavement.

It is obvious that at least two grades of the mineral element, or crushed stone, are essential in order that the stones of the smaller grade may fill the voids between the 35 stones of the larger grade. It has been the most common practice to use three or more grades of crushed stone, but I have devised a combination of two grades of certain relative weights which if mixed according to 40 the proportions which I have devised will form a mass in which the heavier or "wearing stones" will bear the brunt of traffic while the stones of the lighter grade will serve as keys to keep the "wearing stones" 45 in place, thus giving stability to the mass, and enabling the bituminous cement to unite with the whole so as to produce a watertight surface without the use of a large amount of bitumen which is the most expensive of the elements forming this concrete. I am aware that pavements of bituminous concrete have been constructed in which the mineral aggregate was of two 50 grades, but the peculiarity of my pavement lies in the relative weights of the stones used and the relative amount of each grade in the

mixture whereby are effected both stability and economy of materials and labor.

The construction can easily be understood by reference to the drawings, in which— 60

Figure 1 is a view in section representing a part of a sheet street pavement containing my invention, the sub-foundation being of concrete. Fig. 2 is a similar but enlarged view showing a sub-foundation of rolled stones of different sizes. Fig. 3 is an enlarged view in section of the wearing surface to show its construction.

Referring to the drawings:—A is the wearing surface shown more in detail in Fig. 3.

B is the foundation which might be of any desired kind, section b<sup>1</sup>, Fig. 1, showing concrete, while b<sup>2</sup>, Fig. 2, shows rolled broken stones.

a<sup>1</sup> are the "wearing stones" (see Fig. 3) in contact with each other. These stones take the entire impact wear and tear of the traffic and might be of any desirable weight or size.

a<sup>2</sup>, Fig. 3, shows the "filling stones" in their places. These stones are of most importance in my construction and upon them hinge the novelty of this invention. Each of these stones should have a weight which is to the weight of a "wearing stone" as 1:40—50, or weight approximating 2% to 2½% of the weight of each "wearing stone", the actual weight of the different particles depending somewhat upon the fracture into which different kinds of stone break; stones like trap or granite breaking into cubes require such a ratio as 1:40, or about 2½% of the weight of a "wearing stone," while limestones, slate, etc., which break into slabby pieces, require the ratio of 1:50, or about 2% of the weight of a "wearing stone".

Of these "filling stones" having the above ratio I use an amount by weight which is to the "wearing stones" about as 1:2; for instance, if "wearing stones" the individual pieces of which weigh 50 grams are used, I take of these stones two parts and add to them one part by weight of filling stones the individual pieces of which weigh about one gram, the amount of the one gram "filling stones" is sufficient to enter all spaces between the "wearing stones", which are in contact, and key and fill the same.

a<sup>3</sup>, Fig. 3, shows the bituminous cement mixed with sand or other fine mineral to cement and fill the remaining spaces and bind

the whole into a mass. It can readily be seen that latitude in the proportion is necessary as the same depends upon the fracture and shape into which different kinds of stones are crushed. In some cases the ratio of the "filling stones" to the "wearing stones" might be as 2:3 and in others might be as 1:3, but under ordinary conditions the ratio will be 1:2. It should be understood that this wearing surface is applied to the sub-foundation while the bituminous composition is in a plastic condition and under moderate or heavy pressure preferably provided by steam rollers. It will also be understood that the pavement is adapted for any purpose where a continuous sheet covering is necessary in roadways, sidewalks, areas, etc. Having thus fully described my invention, I claim and desire to secure by Letters Patent of the United States:—

1. A wearing surface in a pavement or roadway composed of wearing and filling stones the ratio of the weight of each filling stone to the weight of each wearing stone being approximately as 1:50, the wearing stones being in contact with each other the

smaller stones serving as keys to the larger stones and the whole being mixed with a bituminous cement as described.

2. A wearing surface in a pavement or roadway composed of wearing and filling stones, the amount of filling stones being proportioned to the wearing stones by weight in a ratio approximately 1:2, the smaller stones serving as keys to the larger stones and the whole being bound with a bituminous material as described.

3. A wearing surface in a pavement or roadway composed of wearing and filling stones, each of the filling stones having a weight which is to the wearing stones approximately in the ratio of 1:50 and the quantity by weight of filling stones being proportioned to the wearing stones in approximately the ratio of 1:2, the smaller stones serving as keys to the larger stones and the whole being bound by a bituminous cement as described.

AUGUST E. SCHUTTE.

In the presence of—

ROBERT E. BREWER,  
M. V. FOLEY.